

(No Model.)

F., R. & O. KAMPFE.

EMERY WHEEL FOR WET GRINDING.

No. 351,180.

Patented Oct. 19, 1886.



WITNESSES:

F. W. Rosenbaum.  
Carl Karp

INVENTORS  
Frederick Kampfe, Richard  
Kampfe and Otto Kampfe  
by George Reganur  
ATTORNEYS.

# UNITED STATES PATENT OFFICE.

FREDERICK KAMPFE, RICHARD KAMPFE, AND OTTO KAMPFE, OF BROOKLYN, NEW YORK.

## EMERY-WHEEL FOR WET GRINDING.

SPECIFICATION forming part of Letters Patent No. 351,180, dated October 19, 1886.

Application filed March 12, 1886. Serial No. 194,941. (No model.)

*To all whom it may concern:*

Be it known that we, FREDERICK KAMPFE, RICHARD KAMPFE, and OTTO KAMPFE, of Brooklyn, Kings county, New York State, have invented certain new and useful Improvements in Emery-Wheels for Wet Grinding, of which the following is a specification.

The great objection to all the emery-wheels used heretofore has been that the emery crystals are not held and bound together with sufficient firmness and are apt to be broken from the wheel, this being especially the case with the larger crystals, whereby the grinding edge or face of the wheel is rendered jagged and uneven in a short time and the wheel cannot be used for fine grinding.

The object of our invention is to provide a new and improved emery-wheel in which the emery crystals are held firmly and the spaces between them are filled, thus preventing the working edge or face of the wheel from becoming rough or uneven.

The invention consists in an emery-wheel composed of a mixture of emery, sulphur, and pulverized clay, chalk, or other earthy material.

In the accompanying drawing a perspective view of our improved emery-wheel is shown.

In making the wheel we melt a quantity of sulphur and add to the molten sulphur the pulverized emery and pulverized clay, chalk, or any other earthy material, the emery and earthy material being about equal in quantity.

ties. The ingredients are thoroughly mixed and then pressed into suitable molds and permitted to harden. The sulphur binds the particles of emery and earthy material, and the mixture of sulphur and finely-pulverized earthy material fills the interstices between the crystals of emery, and thus smooth working-surfices are formed. The sulphur alone is too brittle to hold the emery crystals. The finely-pulverized earthy material gives the sulphur greater tenacity, and fills the interstices between the emery crystals perfectly. The particles of earthy material, sulphur, and emery worn off during the grinding operation are washed off by the water delivered upon the wheel during the operation of grinding.

Having thus described our invention, we claim as new and desire to secure by Letters Patent—

As an improved article of manufacture, an emery-wheel for wet grinding, composed of emery, molten sulphur, and pulverized chalk mixed, united, and molded, substantially as set forth.

In testimony that we claim the foregoing as our invention we have signed our names in presence of two subscribing witnesses.

FREDERICK KAMPFE.

RICHARD KAMPFE.

OTTO KAMPFE.

Witnesses:

WILBUR RANKIN,

ALAN D. KENYON.